

1

3,330,765  
POWDERLESS ETCHING BATH AND  
METHOD OF ETCHING

Clayton W. Hoornstra, Midland, Mich., assigner to The Dow Chemical Company, Midland, Mich., a corporation of Delaware  
No Drawing. Filed Oct. 1, 1965, Ser. No. 492,258  
7 Claims. (Cl. 252—79.4)

This application is a continuation-in-part of a copending application Ser. No. 286,510, filed June 10, 1963, now abandoned.

The invention relates to an improved etching bath for powderless etching and the method of etching printing plates, name plates, templates and the like with the improved bath.

In the conventional method of making a metal printing surface, such as a photoengraving, a plate of an acid-soluble metal such as magnesium, zinc and their alloys is coated with a light-sensitive coating or enamel which is applied to the metal surface which is usually flat or cylindrical. The coated surface is exposed to light through a negative having an image thereon so as to produce a corresponding image in the coating. The exposed coating surface is "developed" forming an acid-resistant coating in the form of the image produced by the exposure. This acid-resistant coating is further hardened by heating and the image-bearing surface of the plate is then subjected to etching by an acid. As the etching proceeds, the acid tends to etch laterally and undercut the resist and thus distort the image. The standard method of preventing or reducing this undercutting at one time was to "powder" the plate, a time-consuming and difficult operation. This method has now been replaced by the use of so-called "powderless" etching baths which provide for highly selective metal removal in considerable contrast to the uniform metal removal of metal sizing baths or the uniform minimal metal removal of pickling baths.

Heretofore, the acid constituent of powderless etching baths has consisted entirely, or almost entirely, of nitric acid. The use of such acid is accompanied by the evolution of irritating and toxic fumes. Attempts have been made to use hydrochloric acid but these have been largely limited to methods in which the "powder" method of reducing undercutting has been employed.

It is, therefore, a principal object of the present invention to provide an etching bath which does not produce irritating and toxic fumes during the etching process.

Another object of the invention is to provide a less expensive powderless etching bath than a bath employing nitric acid.

Another object of the invention is to provide a powderless etching method which permits avoiding the use of nitric acid.

A further object of the invention is to provide a suitable powderless etching bath employing hydrochloric acid as the etching agent.

These and other objects and advantages of the present invention will be more fully understood upon becoming familiar with the following description and the appended claims.

It has been discovered that upon combining (1) an etching agent consisting of hydrochloric acid with (2) an organic, water-immiscible liquid comprising at least 65 percent by volume of a member of the group consisting of aromatic hydrocarbons and derivatives thereof having an aromatic nucleus and being predominantly aromatic in character, and mixtures thereof, and the balance, if any, being a water-immiscible organic solvent, said organic water-immiscible liquid being substantially immiscible with water and substantially non-reactive with the etching agent and the metal to be etched, and with (3) one or

2

more filming agents selected from the group consisting of sulfonated or sulfated anionic surface active agents possessing solubility in both water and the organic water-immiscible liquid employed, in concentrations hereinafter more particularly described, and (4) the balance being water, and the etching bath being maintained in an emulsified condition a powderless etching bath is provided which is suitable for photoengraving and for etching printing plates, name plates, templates and the like, which avoids the disadvantages of the nitric acid baths described above as well as the difficulties encountered in prior attempts to use hydrochloric acid as the etching agent.

An organic compound that is predominantly aromatic in character exhibits the properties of a compound in which the characteristics of the resonant ring structure predominate, especially as to solvency behavior.

Suitable amounts of hydrochloric acid employed are here defined most conveniently in terms of the concentrated acid of commerce, although it is obvious larger volumes of more dilute aqueous acid containing corresponding weights of hydrogen chloride may be used. Concentrated hydrochloric acid consists of about 37.5 percent hydrogen chloride by weight. Operable amounts of hydrochloric acid range from 1-25 percent by volume of concentrated hydrochloric acid. A preferred range of hydrochloric acid concentration in the etching bath is from 7-15 percent by volume, in terms of the concentrated acid. If hydrochloric acid concentrations in the bath are too high, the etching rate becomes excessive and the area under the resist in photoengraving plates is poorly protected. If the concentration of hydrochloric acid is too low, not only does the etching rate become very slow, but there is a tendency for open areas to be subject to "blank off," that is, the open area is not etched at all.

The organic, water-immiscible liquid may be a single compound or blend of such compounds. Required properties of this component of the bath are that it be substantially stable in the presence of dilute hydrochloric acid at bath temperatures, that it be a liquid at bath temperatures, and that it have some solvency for the surface active agent. Substantially stable is defined as the non-occurrence of deterioration within a reasonable time period due to the presence of dilute hydrochloric acid which significantly alters the function of the organic water-immiscible liquid within the bath in an unfavorable manner.

The solvency properties of the organic, water-immiscible liquid are further defined by requiring that at least 65 percent by volume, and more preferably at least 90 percent, of such liquid is a member of the group consisting of aromatic hydrocarbons, derivatives thereof having an aromatic nucleus and being predominantly aromatic in character, and mixtures thereof, and up to 35 percent by volume, but preferably not more than 10 percent, of non-aromatic water-immiscible organic solvent.

Suitable aromatic hydrocarbons and derivatives of aromatic compounds when used as substantially pure compounds, and not as mixtures or blends, exhibit a boiling temperature in the range of about 195° to about 735° F. In the case of mixtures of such compounds employed as the organic, water-immiscible liquid, the boiling temperature after distillation of about 10 percent by volume of the liquid is not appreciably below 195° F., while the boiling temperature after distilling off 90 percent by volume of the liquid should be below about 735° F.

Examples of suitable compounds include: diethyl benzenes, tetramethyl benzenes, diisopropyl benzenes, dodecyl benzenes, monochloroethyl benzene, diamyl naphthalene, and aliphatic naphthenics.

Non-aromatic organic solvents which may be used, but only as a part of the organic, water-immiscible liquid, are selected from organic liquids which are substantially immiscible with water, stable in the presence of aqueous

hydrochloric acid at bath temperatures, and liquid at bath temperatures. Preferably not more than about 10 percent by volume of such liquids is employed. In general, it is desirable to avoid alcohols and also aliphatics such as mineral seal oil or white mineral oil, though up to 10 percent of the organic, water-immiscible liquid may consist of such alcohol or high boiling paraffinic oil.

Suitable substantially non-aromatic solvents usable as a part of the organic, water-immiscible liquid include: hexyl acetate, trichloroethylene, ethylbutyl ketone, methylhexyl ketone, isophorone, d-limonene and turpentine. Generally, it may be said that water-immiscible, acid-stable, non-aromatic esters, ketones, terpenes, isoparaffinic hydrocarbons boiling in the range of 200 to 500° F. and ethers may be so employed.

Certain commercial solvents also serve very effectively as the organic water-immiscible liquid component of the bath. An example is a commercial aromatic solvent marketed under the tradename of Solvesso 150, which is a mixture of approximately 90 percent alkyl benzenes, 2 percent naphthalene and 8 percent naphthenes. It has a flash point of 150° F., an aniline point of -18° F., and a distillation temperature range at 760 mm. Hg: initial boiling point of 303° F., 50 percent distilled at 378° F. and dry point at 415° F. Another commercial aromatic solvent suitably employed has the tradename Penola H.A.N. and contains 84 percent aromatics, has a flash point of 140° F., an aniline point of -2° F. and a distillation temperature range at 760 mm. Hg: initial boiling point of 340° F., 50 percent distilled at 446° F. and dry point at 532° F.

Two additional commercial solvents found entirely satisfactory are Panasol AN1 and Panasol AN2 liquids. Both of these solvents consist of more than 90 percent by volume of aromatic hydrocarbons and derivatives thereof.

The amounts of the water-immiscible organic liquid employed may range from 1-10 percent by volume of the bath, but a preferred range is from 3-6 percent by volume.

The hydrophobic-hydrophilic filming agent employed is a compound or blend of compounds selected from the group consisting of sulfonated or sulfated anionic surface active agents possessing solubility in both water and the organic water-immiscible liquid employed in the bath. Suitable types of filming agents include the alkyl aryl sulfonates, esters of sulfosuccinic acid, chlorinated alkyl aryl sulfonates, alkyl aryl ether sulfonates, petroleum sulfonates, sulfonated fatty acid esters, sulfated castor oil or other sulfated natural oils and other surface active agents and mixtures thereof having the requisite solubility in both the organic water-immiscible liquid and water, and exhibiting the requisite filming properties. The filming agent employed must have a solubility, by weight, of at least 0.01 percent in each of water and the organic water-immiscible liquid, and further, must possess a solubility of at least 0.1 percent in at least one of water and the organic water-immiscible liquid. In addition, the filming agent must be entirely taken up between the two phases of the bath, with the preponderance of the filming agent being present in the oil phase of the bath. The suitable filming agents are further defined as having at least 10 carbon atoms in the hydrophobic portion of the molecule. The amounts of the hydrophobic-hydrophilic filming agent employed may range from 0.1 to 5 percent by weight of the bath, but a preferred range is from 0.3 to 4.5 percent by weight.

It is believed that in forming a film, the polar part of the filming molecule attaches to the metal surface while the hydrophobic non-polar segment of the molecule, having an affinity for the organic water-immiscible liquid, draws such atoms to it, thereby perfecting a substantially acid-resistant film. By virtue of the objects to be accomplished, the bath of this invention must have selective filming tendencies under the conditions present

as the etching process is carried out, i.e., acid-resistant films must be formed and retained upon the side walls of the relief but adjacent resist-free areas must be susceptible to the etching action of the hydrochloric acid in a direction normal to the surface of the plate being etched.

Water constitutes the remaining essential component of the bath. It is to be noted, however, that in some baths there may be other materials present, particularly by-products from the production of the foregoing components. Alternatively, other materials which enhance a particular effect may be employed.

Thus, in some instances, it has been found beneficial to add to the organic, water-immiscible liquid, as a modifier, a small amount of an ester such as n-hexylacetate. In other instances, it has been found quite beneficial to add small but very effective amounts of nitric acid in order to improve both the etching rate and the etch factor. The amounts of concentrated nitric acid (density 42° Baumé) advantageously employed range from 2 to about 13 percent by volume based on the volume of concentrated hydrochloric acid employed, or, stated in other terms, from about 0.33 to about 2 percent by volume of concentrated nitric acid based on the total volume of the etching bath.

Etch factor as used in this specification is defined as the ratio of the depth of the etch adjacent to a line of resist divided by one-half of the total loss in width (i.e., side etch) of metal immediately beneath the resist.

In the practice of the present invention, it has been found desirable to impinge the bath upon the surface to be etched as by spraying, but much more preferably, by splashing. In the formulation of the etching bath, it has been found to be a general rule that as the concentration of the hydrochloric acid is increased within the aforementioned limitations, it is necessary to also increase the proportion of filming agent employed. It has also been found that the selection of the organic, water-immiscible liquid and of the filming agent are interrelated in that the filming agent must have some solubility in the organic water-immiscible liquid, as defined hereinabove. Due to bath depletion as the etching process is carried out, it is simpler and more convenient to designate amounts of components in terms of their initial concentrations.

Suitable metals which may be etched by this process include zinc, zinc-base alloys, magnesium and magnesium-base alloy, all of which are substantially homogeneous metals suitable for photoengraving. A zinc-base alloy or magnesium-base alloy is defined as having at least 70 percent of the base component.

The average bath temperature may be within a range from 50-120° F., but a preferred range is from 70-90° F. A preferred embodiment of this invention comprises, per liter of bath, about 115 ml. of 37.5 percent by weight hydrochloric acid, about 30 ml. of Solvesso 150 aromatic solvent, about 5 grams of Ninex 300 triethanolamine dodecylbenzene sulfonate and about 15 ml. of 42° Baumé nitric acid. The remainder of the mixture is water.

To carry out the etching process, it is preferred to employ an etching machine of the type disclosed in U.S. Patent 2,669,048, issued Feb. 16, 1954. In this "Dowetch" machine, rotating, elongated paddles intermittently splash the etching bath upwardly against the image-bearing surface of the object being etched. The splashing action of the paddles also serves to keep the bath in an emulsified state. The emulsified bath of this invention applied in the described manner for about 8 minutes will usually produce depths of etch from approximately 0.015 to 0.030 inch in line areas of the plate while generally producing proper depths in various other parts of the plate. Also, etch factors in line image areas from 20 to 40 are readily obtainable. It is obviously desirable to have as high etch factors as possible for faithful reproduction of the image in relief. However, it should be noted that the etch factor can be sensitive to changes in depth. Thus, etch factor should be considered as only one criterion of etching bath quality.

The etching bath of the invention has very good chemical

stability as a function of time and is capable of producing uniform and good results on consecutive plates over periods of many hours.

The following examples are intended to be merely illustrative of the invention and should not be construed as limiting the scope of the invention.

In a series of tests employing the method and composi-

This same procedure was followed throughout the series of tests in which various concentrations of hydrochloric acid, various surface active agents and various amounts of the organic, water-immiscible liquid Solvesso 150 were employed. The amounts and nature of the ingredients employed and the results obtained are summarized in the following table.

TABLE I

| Test No.             | Surface Active Agent                                                  |                    |                                                | Range, ml. Solvesso 150 | Ml. HCl | Typical Etch Factor Range | Line Depth, Mils |
|----------------------|-----------------------------------------------------------------------|--------------------|------------------------------------------------|-------------------------|---------|---------------------------|------------------|
|                      | Name                                                                  | Nature or Identity | Conc. Range, w/w. percent (active ingredients) |                         |         |                           |                  |
| 1. Tensol N.         | Sulfonated Naphthalene Alkyl Ether                                    | 1-2                | 180-360                                        | 700                     | 4-23    | 7-23                      |                  |
| 2. Sulframin N.      | Sodium Diethyl Naphthalene Sulfonate                                  | 0.7                | 330                                            | 850                     | 15-30+  | 10-26                     |                  |
| 3. Ninate 402        | Calcium Dodecylbenzene Sulfonate                                      | 0.4                | 240                                            | 900                     | 12-24   | 12-24                     |                  |
| 4. Ninate 411        | Amine Alkyl Aryl Sulfonate                                            | 0.3                | 120                                            | 700                     | 15      | 23                        |                  |
| 5. Aerosol OT-EG     | Methyl Heptyl Ester of Sodium Salt of Sulfosuccinic Acid              | 0.8                | 180                                            | 950                     | 23      | 16                        |                  |
| 6. Alrowet D65       | Diethyl Sodium Sulfosuccinate                                         | 0.3                | 120-150                                        | 700                     | 15-20   | ca. 30                    |                  |
| 7. (Ninex 300)       | Triethanolamine Dodecylbenzene Sulfonate                              | 0.17               |                                                |                         |         |                           |                  |
| 8. Stepan 164-16     | Highly Sulfonated Fatty Acid Ester plus Span 80 (Sorbitan Monooleate) | 1.5                | 240                                            | 700                     | 19      | 11                        |                  |
| 9. (Monopole Oil 48) | Sulfated Castor Oil                                                   | 0.8                | 540                                            | 850                     | 7       | 10                        |                  |
| (Ricinoleic Acid)    | Sodium Salt of Alkyl Aryl Polyether Sulfate                           | 0.5-1.0            | 240-300                                        | 700                     | 8-19    | 9-12                      |                  |

<sup>1</sup> 60 ml. n-hexyl acetate was added to the Solvesso 150 liquid.

tion of the invention, a powderless etching bath of 6 liters volume was prepared in a miniature "Dowetch" machine by adding requisite quantities of concentrated aqueous hydrochloric acid (37.5 percent by weight HCl), an organic water-immiscible liquid, a surface active agent and water. The filming agent was conveniently first dissolved or dispersed in a small amount of water before adding it to the resulting mixture in the bath. The bath temperature was

30 In an additional series of tests, small amounts of nitric acid were employed in addition to hydrochloric acid. The other conditions of the test were similar to those described for the first series of tests. The amounts of nitric acid and hydrochloric acid employed, the nature and amounts of surface active agent and the quantity of Solvesso 150 liquid employed, as well as the results obtained are summarized in Table II.

TABLE II

| Test No.            | Surface Active Agent                                     |                    |                                                | Range, ml. Solvesso 150 | Ml. HCl | Ml. HNO <sub>3</sub> Added | Typical Etch Factor or Range | Line Depth, Mils |
|---------------------|----------------------------------------------------------|--------------------|------------------------------------------------|-------------------------|---------|----------------------------|------------------------------|------------------|
|                     | Name                                                     | Nature or Identity | Conc. Range, percent w/w. (active ingredients) |                         |         |                            |                              |                  |
| 1. Ninex 300        | Triethanolamine Dodecylbenzene Sulfonate                 | 0.5                | 180                                            | 700                     | 30      | 30-50                      | 17.6                         |                  |
| 2. Alicowet ANS     | Amyl Naphthalene Sodium Sulfonate                        | 2.4                | 570                                            | 900                     | 20      | 22                         | 16                           |                  |
| 3. Beaconal T       | Guamidine Salt of Monoethyl Phenyl Phenol Monosulfonate  | 1.8                | 360                                            | 700                     | 60      | 14.5                       | 14.5                         |                  |
| 4. Aerosol OT (EG)  | Tridecyl Benzene Sulfonate                               | 0.5                | 210                                            | 700                     | 30-60   | 8-16                       | 6                            |                  |
| 5.                  | Methyl Heptyl Ester of Sodium Salt of Sulfosuccinic Acid | 2.0                | 300                                            | 950                     | 120     | 24                         | 18                           |                  |
| 6.                  | Sodium Dodecyl Monochloro Diphenyl Oxide Sulfonate       | 4.5                | 360                                            | 900                     | 90      | 14.6                       | 10                           |                  |
| 7. Petronate L      | Petroleum Sulfonate                                      | 1.0-2.5            | 250-310                                        | 950                     | 30-90   | 6-30+                      | 9-21                         |                  |
| 8. Petronate        | do                                                       | 1.5-2.0            | 300-330                                        | 700                     | 60      | 6-25                       | 7-14                         |                  |
| 9. Triton W-30      | Sodium Salt of Alkyl Aryl Polyether Sulfate              | 0.7                | 300                                            | 700                     | 30      | 10.5                       | 8                            |                  |
| 10. Tetranol        | Sodium Salt of Fatty Acid Ester                          | 0.7                | 270                                            | 700                     | 60      | 11.8                       | 11.8                         |                  |
| 11. Trepanol S-30-T | Sodium Tridecyl Polyglycol Ether Sulfate                 | 0.5                | 210                                            | 700                     | 60      | 8                          | 4                            |                  |

<sup>1</sup> 30 ml. n-hexylacetate added to Solvesso 150 liquid.

adjusted to about room temperature, approximately 72°-75° F., while the circulating pump mixed the bath emulsifying the oily phase into the aqueous phase of the bath. A plate approximately 2" x 3.5" x 0.064", formed of a magnesium-base alloy containing approximately 3 percent Al, 1 percent Zn and trace amounts of impurities, having a light-sensitive polyvinyl alcohol resist thereon was exposed to a standard test pattern of letters, lines, dots and a halftone image, developed and descummed in the manner well known to photoengravers. The plate was descummed by a 2-minute immersion in an aqueous solution consisting of 12 ounces per gallon of potassium hydroxide and 2 ounces per gallon of potassium permanganate, followed by brushing the surface with dilute nitric acid until the surface was bright. The plate was then placed in the etching machine, the paddles were turned on and etching was allowed to continue for about 5 to 10 minutes.

60

65

70

75

In additional runs, made by way of comparison, a number of identical small magnesium photoengraving alloy test plates were prepared by photoprinting thereon both linework and halftone images with a polyvinyl alcohol-chromate type resist by conventional processes. Just before use each plate was descummed by rubbing it vigorously with dry chalk. All etching was done in a miniature "Dowetch" machine wherein each plate was, in turn, mounted horizontally with the image side down and rotated in the splash emanating from the rotating paddles of the machine.

Three liters of 37.5 percent by weight hydrochloric acid and three liters of ordinary non-detergent type SAE 20 weight motor oil were placed in the machine and the paddles were run at 600 revolutions per minute (r.p.m.) for about one minute to form a composition outside the scope of the invention. Two test plates were then etched at

a paddle speed of 600 r.p.m. with the bath at a temperature of 78° F.

The first plate was etched for 10 seconds. The reaction was violent. Image elements 0.009 inch wide or less were completely undermined by lateral etching and were lost though the depth of relief was only 0.002 inch, indicating an etch factor of less than 0.5. The results were completely unsatisfactory.

The second plate was etched for 60 seconds. The etch was 0.011 inch deep and the entire image was undermined and etched away, showing that the bath was completely unsuitable.

900 milliliters of 37.5 percent by weight hydrochloric acid and 240 milliliters of SAE 20 weight motor oil were placed in a miniature etching machine and the balance of the 6 liter bath was made up with water. The paddles were run at 600 r.p.m. for one minute before etching was begun on magnesium test plates having a photoresist image developed thereon.

A first plate was etched for 6 minutes, while a second plate was etched for 90 seconds. Extremely rapid, substantially non-selective etching took place on both plates.

The foregoing bath was modified by the addition of 360 milliliters more SAE 20 weight motor oil, bringing the proportion of oil in the bath to 10 percent by volume.

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

the metal to be etched, and (4) a liquid at bath temperatures; and said filming agent being further characterized as containing at least 10 carbon atoms in the hydrophobic portion of the molecule, and having a solubility, by weight, of at least 0.01 percent in each of the water and the organic, water-immiscible liquid.

2. An emulsified powderless etching bath consisting essentially of 1 to 25 percent by volume of 37.5 percent by weight hydrochloric acid; 1 to 10 percent by volume of an organic, water-immiscible liquid; 0.1 to 5 percent by weight of a hydrophobic-hydrophilic filming agent selected from the group consisting of sulfonated organic compounds and sulfated organic compounds; and the balance being water; said organic, water-immiscible liquid comprising at least 90 percent by volume of a member of the group consisting of an aromatic hydrocarbon, a derivative of an aromatic hydrocarbon having an aromatic nucleus and being predominantly aromatic in character, and mixtures thereof, and up to 10 percent by volume of a water-immiscible organic solvent, said organic, water-immiscible liquid being (1) substantially stable in the said bath at a temperature in the range of 50-120° F., (2) substantially immiscible with the water, (3) substantially non-reactive with the hydrochloric acid and the metal to be etched, and (4) a liquid at bath temperatures; and said filming agent being further characterized as containing at least 10 carbon atoms in the hydrophobic portion of the molecule, and having a solubility, by weight, of at least 0.01 percent in each of the water and the organic, water-immiscible liquid.

3. An emulsified powderless etching bath consisting essentially of 7 to 15 percent by volume of 37.5 percent by weight hydrochloric acid; 1 to 10 percent by volume of an organic, water-immiscible liquid; 0.1 to 5 percent by weight of a hydrophobic-hydrophilic filming agent selected from the group consisting of sulfonated organic compounds and sulfated organic compounds; and the balance being water; said organic, water-immiscible liquid comprising at least 65 percent by volume of a member of the group consisting of an aromatic hydrocarbon, a derivative of an aromatic hydrocarbon having an aromatic nucleus and being predominantly aromatic in character, and mixtures thereof, and up to 35 percent by volume of a water-immiscible organic solvent, said organic, water-immiscible liquid being (1) substantially stable in the said bath at a temperature in the range of 50-120° F., (2) substantially immiscible with the water, (3) substantially non-reactive with the hydrochloric acid and the metal to be etched, and (4) a liquid at bath temperatures; and said filming agent being further characterized as containing at least 10 carbon atoms in the hydrophobic portion of the molecule, and having a solubility, by weight, of at least 0.01 percent in each of the water and the organic, water-immiscible liquid.

4. An emulsified powderless etching bath consisting essentially of 1 to 25 percent by volume of 37.5 percent by weight hydrochloric acid; from 0.33 to 2 percent by volume of 42° Baumé nitric acid; 1 to 10 percent by volume of an organic, water-immiscible liquid; 0.1 to 5 percent by weight of a hydrophobic-hydrophilic filming agent selected from the group consisting of sulfonated organic compounds and sulfated organic compounds; and the balance being water; said organic, water-immiscible liquid comprising at least 65 percent by volume of a member of the group consisting of an aromatic hydrocarbon, a derivative of an aromatic hydrocarbon having an aromatic nucleus and being predominantly aromatic in character, and mixtures thereof, and up to 35 percent by volume of a water-immiscible organic solvent, said organic, water-immiscible liquid being (1) substantially stable in the said bath at a temperature in the range of 50-120° F., (2) substantially immiscible with the water, (3) substantially non-reactive with the hydrochloric acid

and the metal to be etched, and (4) a liquid at bath temperatures; and said filming agent being further characterized as containing at least 10 carbon atoms in the hydrophobic portion of the molecule, and having a solubility, by weight, of at least 0.01 percent in each of the water and the organic, water-immiscible liquid.

5. An emulsified powderless etching bath consisting essentially of 7 to 15 percent by volume of 37.5 percent by weight hydrochloric acid; 3 to 6 percent by volume of an organic, water-immiscible liquid; 0.3 to 4.5 percent by weight of a hydrophobic-hydrophilic filming agent selected from the group consisting of sulfonated organic compounds and sulfated organic compounds; and the balance being water; said organic, water-immiscible liquid comprising at least 90 percent by volume of a member of the group consisting of an aromatic hydrocarbon, a derivative of an aromatic hydrocarbon having an aromatic nucleus and being predominantly aromatic in character, and mixtures thereof, and up to 10 percent by volume of a water-immiscible organic solvent, said organic, water-immiscible liquid being (1) substantially stable in the said bath at a temperature in the range of 50-120° F., (2) substantially immiscible with the water, (3) substantially non-reactive with the hydrochloric acid and the metal to be etched, and (4) a liquid at bath temperatures; and said filming agent being further characterized as containing at least 10 carbon atoms in the hydrophobic portion of the molecule, and having a solubility, by weight, of at least 0.01 percent in each of the water and the organic, water-immiscible liquid.

6. A method of etching the surface of an acid-soluble metal plate having an acid-resistant, partial coating thereon, said metal being selected from the group consisting of zinc, zinc-base alloys, magnesium and magnesium-base alloys which comprises: repeatedly impinging upon the metal surface to be etched an emulsified powderless etching bath consisting essentially of from 1 to 25 percent by volume of 37.5 percent by weight hydrochloric acid; 1 to 10 percent by volume of an organic, water-immiscible liquid; 0.1 to 5 percent by weight of a hydrophobic-hydrophilic filming agent selected from the group consisting of sulfonated organic compounds and sulfated organic compounds; and the balance being water; said organic, water-immiscible liquid comprising at least 65 percent by volume of a member of the group consisting of an aromatic hydrocarbon, a derivative of an aromatic hydrocarbon having an aromatic nucleus and being predominantly aromatic in character, and mixtures thereof, and up to 35 percent by volume of a water-immiscible organic solvent, said organic, water-immiscible liquid being (1) substantially stable in the said bath at a temperature in the range of 50-120° F., (2) substantially immiscible with the water, (3) substantially non-reactive with the hydrochloric acid and the metal to be etched, and (4) a liquid at bath temperatures; and said filming agent being further characterized as containing at least 10 carbon atoms in the hydrophobic portion of the molecule, and having a solubility, by weight, of at least 0.01 percent in each of the water and the organic, water-immiscible liquid.

7. A method of etching the surface of an acid-soluble metal plate having an acid-resistant, partial coating thereon, said metal being selected from the group consisting of zinc, zinc-base alloys, magnesium and magnesium-base alloys which comprises: repeatedly impinging upon the metal surface to be etched an emulsified powderless etching bath consisting essentially of 1 to 25 percent by volume of 37.5 percent by weight hydrochloric acid; from 0.33 to 2 percent by volume of 42° Baumé nitric acid; 1 to 10 percent by volume of an organic, water-immiscible liquid; 0.1 to 5 percent by weight of a hydrophobic-hydrophilic filming agent selected from the group consisting of sulfonated organic compounds and sulfated organic compounds; and the balance being water; said

organic, water-immiscible liquid comprising at least 65 percent by volume of a member of the group consisting of an aromatic hydrocarbon, a derivative of an aromatic hydrocarbon having an aromatic nucleus and being predominantly aromatic in character, and mixtures thereof, and up to 35 percent by volume of a water-immiscible organic solvent, said organic, water-immiscible liquid being (1) substantially stable in the said bath at a temperature in the range of 50-120° F., (2) substantially immiscible with the water, (3) substantially non-reactive with the hydrochloric acid and the metal to be etched, and (4) a liquid at bath temperatures; and said filming agent being further characterized as containing at least 10 carbon atoms in the hydrophobic portion of the molecule, and having a solubility, by weight, of at least 0.01 percent in each of the water and the organic water-immiscible liquid.

## References Cited

## UNITED STATES PATENTS

|   |           |         |                |       |            |
|---|-----------|---------|----------------|-------|------------|
| 5 | 1,918,545 | 7/1933  | Hoy            | ----- | 252—79.2 X |
|   | 2,828,194 | 3/1958  | Hopkins et al. | ----- | 252—79.2 X |
|   | 3,023,138 | 2/1962  | Easley et al.  | ----- | 252—79.4   |
|   | 3,074,836 | 1/1963  | Sherer et al.  | ----- | 252—79.4 X |
|   | 3,105,783 | 10/1963 | Parkinson      | ----- | 156—14     |
|   | 3,193,423 | 6/1965  | Goffredo       | ----- | 252—79.2 X |

10

## FOREIGN PATENTS

778,901 7/1957 Great Britain.

LEON D. ROSDOL, Primary Examiner.

15 ALBERT T. MEYERS, Examiner.

M. WEINBLATT, Assistant Examiner.